

May 27, 1958

J. A. LORITSCH ET AL

2,836,518

MODIFIED POLYVINYL ACETAL INSULATED CONDUCTORS

Filed Dec. 7, 1953



Inventors:  
John A. Loritsch,  
Edward W. Daszewski,  
by *Allen G. G.*  
Their Attorney.

1

2,836,518

## MODIFIED POLYVINYL ACETAL INSULATED CONDUCTORS

John A. Loritsch and Edward W. Daszewski, Schenectady, N. Y., assignors to General Electric Company, a corporation of New York

Application December 7, 1953, Serial No. 396,582

6 Claims. (Cl. 117—232)

This application is a continuation-in-part of our co-pending application Serial No. 376,620, filed August 26, 1953, now abandoned, and assigned to the assignee of the present invention.

This invention relates to resinous compositions and conductors insulated therewith. More particularly, the invention is concerned with improved enamels comprising polyvinyl acetals and to electrical conductors provided with such enamels.

Patnode and Flynn Patent 2,085,995, assigned to the assignee of the present invention, discloses insulated conductors provided with coating compositions comprising polyvinyl acetal resins. Although such insulated conductors have distinct advantages over conductors insulated with conventional oil-type enamels, the resinous compositions utilized therein are costly, and comparatively high priced solvents are required for the production of suitable wire enamels therefrom. Jackson and Hall Patent 2,307,588, also assigned to the assignee of the present invention, discloses insulated conductors provided with an improved and less expensive resinous composition which additionally is soluble in relatively inexpensive solvents. Accordingly, insulated conductors having properties practically the same, and in certain respects even better than those described in the above Patnode et al. patent, can be made and at a substantially lower cost by combining suitable phenol-aldehyde resins with the polyvinyl acetal resin. Although conductors insulated with the Jackson and Hall compositions are eminently satisfactory for most applications, they do not possess the required solvent resistance necessary in certain instances, for example, when used in hermetically sealed motors of refrigerators. The attainment of adequate solvent resistance in addition to abrasion and heat resistance, as well as dielectric strength and other qualities possessed by the aforementioned Patnode and Flynn, and Jackson and Hall compositions has presented a problem, particularly to the magnet wire industry.

In accordance with the present invention, all of the useful advantages of the Patnode and Flynn, and Jackson and Hall compositions and insulated conductors are retained and markedly improved solvent resistance attained, by incorporating in polyvinyl acetal-phenol-aldehyde compositions, a condensate derived from the reaction of an aldehyde with an amino compound, namely, an ammonia derivative. The addition of a small amount, e. g., from 0.1% to 5%, by weight, imparts unexpectedly improved solvent resistance to the compositions and particularly to conductors or wires coated therewith.

The invention will be understood more readily from the following description when considered in connection with the accompanying drawing in which the single figure is a cross-sectional view of an electrical conductor provided with insulation in accordance with this invention.

The aldehyde-ammonia derivative condensates which are useful as additives herein are condensates formed by the known reaction of aldehydes, and particularly formal-

2

dehyde, with ammonia derivatives including amines and amides and, more particularly, with ureas and thioureas, etc., to form, e. g., urea-aldehyde condensates in the usual manner. Thus, aldehyde-amine and aldehyde-amide condensates are produced by the reaction of urea, thiourea and various substituted ureas and urea derivatives with aldehydes such as formaldehydes to form condensates, e. g., methylol ureas, etc. Various other amines and amides can similarly be reacted in known manner with formaldehyde, etc., to form condensates which are amine-aldehyde or amide-aldehyde resins or condensates.

The aldehyde-ammonia derivative condensates found eminently suitable for improving the solvent resistance of phenolic modified polyvinyl acetal compositions are the soluble condensates, i. e., the condensates which are soluble with and compatible with the resin composition. Condensates having these properties and coming within the scope of the present invention are believed to have the grouping



wherein R is a radical of the class consisting of hydrogen, alkyl, aryl, alkaryl, aralkyl, a hetero oxygen-containing radical, for example, furyl



and R' is a radical of the class consisting of hydrogen,



alkyl, aryl, alkaryl, aralkyl, a pyrrole residue, for example,



and



R in the second group having the same scope as in the first group, and n is an integer equal to or greater than one.

Included also are condensates of aldehydes and ammonia derivatives, particularly urea-aldehyde condensates, prepared in the presence of alcoholic or other solvents which take part in the reaction and thus become an integral part of the resulting resin composition, as where butyl alcohol is present in the production of urea formaldehyde condensates to give butylated products.

The polyvinyl acetal resins employed in the process of this invention are hydrolyzed, polymerized vinyl ester aldehyde condensation products which may be produced from various aldehydes and various polyvinyl esters as more fully set forth in said Patnode et al. patent, and more fully described in Reissue Patent 20,430 to Morrison et al.

Aldehydes other than formaldehyde may be used in making polyvinyl acetal resins, for example, acetaldehyde, propionic aldehyde, butyric aldehyde, benzaldehyde and the like. Likewise, polyvinyl esters other than polyvinyl acetate may be employed, for instance, polyvinyl propionate, polyvinyl butyrate and the like. The properties of polyvinyl acetal resins may be varied through a wide range by varying the viscosity and the extent of the hydrolysis of the polyvinyl ester, the amount and the character of the aldehyde reacted with the hydrolyzed poly-

merized vinyl ester, and the character and the amount of the acid catalyst used.

In order that those skilled in the art better may understand how this invention may be carried into effect, the following examples are given to illustrate the preparation of phenolic-modified polyvinyl acetal enamels where in an ammonia derivative-aldehyde condensate is employed to improve the solvent resistance of the enamel. In order to show the improved solvent resistance, the prepared enamels were used to coat wires and four lengths of each coated wire approximately 2 feet long were immersed in boiling solvent mixture to test their solvent resistance. As previously mentioned, one of the end uses of wires insulatingly coated with resinous compositions of the present type is in hermetically sealed motors used in refrigerators where it is subject to the deleterious action of refrigerants such as Freon. Test methods involving the effects of Freon per se on insulation are long and tedious requiring special apparatus. Through a series of tests, it was found that there was a correlation between the effects of a fifty-fifty mixture of solvents such as ethanol and toluene upon insulation of the present description and the action thereon of Freon. This test was more severe than any other conditions which similarly insulated wires may encounter in use. Due to the ease of testing and the closeness in effect of such a mixture to that of Freon, a fifty-fifty mixture of ethanol and toluene was used in all of the tests which follow.

This test involved immersing the lengths of wires in a boiling mixture of 50 parts of alcohol, for example, ethanol, and 50 parts of toluene for a total of 10 minutes, after which time the wires were inspected for signs of visible attack.

In the following examples, given by way of illustration and not by way of limitation, all parts and percentages are by weight.

#### Example 1

| A resin having a solids content of 16% composed of: |                   |
|-----------------------------------------------------|-------------------|
|                                                     | Percent by weight |
| Cresol-formaldehyde resin <sup>1</sup>              | 5.33              |
| Polyvinyl formal resin                              | 10.67             |
| Solvents, 84% formal composed of—                   |                   |
| Cresol <sup>2</sup>                                 | 25.20             |
| Naphtha                                             | 58.80             |

<sup>1</sup> A phenol-aldehyde resin of the type disclosed in Jackson et al. Patent 2,307,588 which disclosure is incorporated herein by reference.

<sup>2</sup> A part of this cresol is added to the dehydrated resin in the reaction vessel.

The proper amounts of naphtha and cresol were weighed into a mixing tank and agitated, a 50-50 cresol solution of cresol-formaldehyde resin added, and the whole well mixed. The solid polyvinyl formal resin was added slowly, and the mixture stirred until the polyvinyl formal resin was completely dissolved. To the resulting enamel was added 1.2%, by weight, based on the weight of the resin solids represented by the polyvinyl formal resin, of a butylated urea-formaldehyde condensate having the probable structure



wherein  $n$  is greater than one. The butylated urea-formaldehyde condensate was an alcoholic type of urea-formaldehyde resin resulting from the reaction of the resin with an alcohol (trade name Uformite 240-N). The resulting composition was agitated with a stirrer for approximately one hour to insure good blending. It may be dyed, if desired, by adding a small amount of a suitable dye during the stirring. Preferably, the enamel is filtered through a pressure filter prior to use for enameling wire.

This enamel was used to coat .0508" wire at various speeds ranging from 14 feet per minute to 21 feet per minute to give an insulation thickness of 5 to 6 mils and was then tested for solvent resistance in accordance with the aforescribed test. In each case, the solvent resistance was excellent.

#### Example 2

To the enamel of Example 1, 1.2%, by weight, based on the weight of resin solids represented by the polyvinyl formal resin, of trimethylol urea having the formula



was added in place of the butylated urea-formaldehyde condensate and the composition processed and tested for solvent resistance as in Example 1. Again in each case, the solvent resistance was excellent.

#### Example 3

To the enamel of Example 1 were added in lieu of the butylated urea-formaldehyde condensate, various amounts of a pyrrole-formaldehyde condensate prepared by reacting formaldehyde with pyrrole in approximately equimolecular proportion having the formula



wherein  $n$  is greater than one, specifically from 0.3 to 1.2%, by weight, based on the weight of resin solids represented by the polyvinyl formal resin, and each composition processed and solvent tested as in Example 1. The solvent resistance of each of the enamels tested was excellent.

#### Example 4

Various enamels were prepared, containing from 0.3 to 1.2%, by weight, based on the weight of resin solids represented by the polyvinyl formal resin, using the enamel composition of Example 1, but employing hexamethylenetetramine in place of butylated urea-formaldehyde condensate. These enamels were used to insulate wire at speeds ranging from 14 to 21 feet per minute and each of the insulated wires was solvent tested in the aforescribed manner. In each case, the solvent resistance was excellent.

#### Example 5

To the enamel of Example 1 was added in place of the butylated urea-formaldehyde condensate 0.3%, by weight, based on the weight of resin solids represented by the polyvinyl formal, of an aniline-formaldehyde condensate prepared by dissolving 100 parts of aniline in 500 parts of 95% alcohol and refluxing with 90 parts of 37% formaldehyde.

The resulting enamel was processed and its solvent resistance tested as in Example 1 and again the solvent resistance was excellent.

#### Example 6

Using the same composition and the same proportions of condensate as in Example 5, an aniline-acetaldehyde condensate prepared in similar manner was substituted and the resulting enamel solvent tested as in previous examples. This enamel also proved to have excellent solvent resistance.

While the invention has been described with particular reference to cresol as the phenolic ingredient in the modified polyvinyl acetal resins, it will be obvious to those skilled in the art that other phenolic bodies also

may be used, for example, those disclosed in Jackson et al. Patent 2,307,588, hereinabove incorporated by reference. Included are xylenols, mixtures of phenol and cresol or mixtures of phenol or cresol or phenol and cresol together with wood oil phenolic bodies of the kind described more fully in Patent No. 2,221,511 to Fiedler et al., dated November 12, 1940, and assigned to the same assignee as the present invention. Additional examples include the petrol-alkyl type phenols, which petro-alkyl phenols may be used as the sole phenolic body or in combination with coal-tar phenol, cresols and other phenolic substances. Likewise, active methylene-containing bodies other than formaldehyde may be used, either in solid or solution state.

The properties of the phenol-aldehyde resin and accordingly the properties of the additive modified phenol-aldehyde-polyvinyl acetal resinous compositions may be varied by varying the ratios of the phenolic body and the aldehyde. For example, resins containing 0.7 or more mols formaldehyde will convert to a substantially infusible insoluble state when heated at elevated temperatures whereas those containing 0.5 or 0.6 mol formaldehyde are thermoplastic. While for certain applications such thermoplastic resins may be used as modifying agents of the polyvinyl acetal resin in general, it is preferred to use in the preparation of wire enamels those phenolic resins which are produced by reacting 1 mol phenolic body with from 0.7 to 2.0 mols of an active methylene-containing body such as formaldehyde or other suitable aldehyde. No particular advantage is gained by using more than 2 mols formaldehyde to 1 mol of the phenolic body since the excess formaldehyde is volatilized during the cooking of the resin.

Enamelled wires are produced by drawing the clean wire, for example, clean copper wire through a bath of wire enamel made by incorporating the modifying phenol-aldehyde resin, polyvinyl acetal resin, solvent and ammonia derivative-aldehyde condensate. The proportions of phenolic and polyvinyl acetal resins may be varied, for example, from, by weight, about 5 to 50 parts phenolic resins to form about 95 to 50 parts polyvinyl acetal resin. The total resin to solvent proportions also may be varied, for instance, from about 5 to 25 parts resin to about 95 to 75 parts solvent. It is preferred to use a phenolic resin-polyvinyl acetal resin ratio and a total resin-solvent ratio such as described under Example 1, since the particular combination of ingredients there described has been found to produce a wire enamel which is more readily and effectively applied to wire, and to yield an insulated wire having the most desirable combination of properties.

The concentrations of aldehyde-ammonia derivative condensate additive to phenolic resin modified polyvinyl acetal enamels found suitable to improve solvent resistance in accordance with the present invention is wide. Excellent results have been obtained by employing 0.1% to 5%, by weight, based on the weight of resin solids represented by the polyvinyl acetal resin. A preferred range is from 0.3 to 1.2%, by weight, based on the weight of resin solids represented by the polyvinyl acetal resin employed.

Various other solvents are equally as effective in the preparation of the herein-described enamels and are essentially the solvents disclosed in the aforesaid Jackson et al. patent.

The ammonia derivative-aldehyde condensates coming within the scope of the present invention are those which are substantially completely soluble in the enamel and compatible therewith. Condensates which are not soluble or only slightly soluble or which are incompatible with the enamel are ineffective for the present purposes. Although the invention has been described more fully in connection with the specific ammonia derivative-aldehyde condensates of the examples, it is not limited thereto. Any ammonia derivative-aldehyde condensate which

is substantially completely soluble and compatible with the enamel and which generally has the previously defined grouping

5



may be employed. Illustrative examples of aldehydes condensable with an ammonia derivative to give the present condensates include, in addition to the formaldehyde and acetaldehyde of the examples, for instance, propionaldehyde, n-butylaldehyde, isobutylaldehyde, n-valeraldehyde, isovaleraldehyde, n-caproaldehyde, etc., benzaldehyde and the like.

10 The method of coating the aforescribed wires was in accordance with the procedure disclosed in the Jackson et al. patent. For example, after the wire had been passed through a bath containing the particular wire enamel, the coated wire was subjected to heat by introducing it into a suitable oven wherein the enamel was baked at a suitable temperature, for example, at an oven temperature of about 250° to 500° C. The coating was baked simultaneously with the annealing of the copper. As 20 previously mentioned, the wire was drawn through the bath at various speeds ranging from 14 feet per minute to 21 feet per minute. Usually, it was necessary to run the wire successively through the enamel bath and baking oven several times at a constant speed in order to provide adequate insulation thereon. Baking at the previously 25 mentioned temperatures advanced the phenol-aldehyde component of the mixed or combined resin film to the insoluble infusible state, and likewise improved the properties of the polyvinyl acetal resin component. The hardness, abrasion resistance, and resistance of the resin film to attack by oils, solvents, varnishes and various chemicals were improved by such treatment. Wires coated with the instantly described enamels gave results comparable with those resulting from the tests described and illustrated in Patent No. 2,307,588 on the phenol-aldehyde modified polyvinyl acetal enamels therein described. However, there was a substantial improvement 30 in the solvent resistance of the present enamels. Whereas the prior enamel failed completely under the solvent resistant tests hereinbefore described, each of the present enamels containing a condensate of an ammonia derivative and an aldehyde showed excellent solvent resistance under the same conditions. Additionally, it should be noted that the solvent resistant test employed in the instant process is a far more vigorous test than that of the 35 aforementioned patent.

40 It is to be understood that this invention is not limited to the application of the new insulating composition directly upon the conductor as illustrated in the accompanying drawing but may also be applied in accordance with the methods described and illustrated in the Jackson et al. patent.

45 Although the phenolic resin modified polyvinyl acetal resin having incorporated therein an ammonia derivative-aldehyde condensate is particularly applicable to the manufacture of wire enamels and insulated conductors, it will be appreciated that its field of utility is not limited thereto. For example, it may be used to improve the solvent resistance of phenolic resin-modified polyvinyl acetal resin heretofore used as an adhesive 50 for cementing together such materials as mica flakes to form bonded mica sheet insulation, as a cementing agent to bond together fibrous materials in sheet, tape, felted, or other form and as a coil impregnating varnish.

55 The additive containing phenolic resin modified polyvinyl acetal resins may be made in the form of solvent resistant thin sheets or tapes and used alone or adhesively bonded to, or otherwise in combination with, other materials such as paper, cellulose, esters, cellulose ethers, etc., as coil layer insulation. Such sheets or tapes having improved solvent resistance also may be applied to a

conductor, according to well-known strip covering methods, as insulation therefor. They may be heat-treated to improve their properties either before, during or after application.

What we claim as new and desire to secure by Letters Patent of the United States is:

1. An insulated copper conductor in which the outer insulation therefor comprises essentially a hard, flexible, tough, abrasion-resistant and Freon-resistant coating, said coating being the heat-treated product of a mixture of ingredients consisting essentially, by weight, of (1) from 95 to 50 percent of a polyvinyl formal resin obtained by condensing formaldehyde with a product of hydrolysis of polyvinyl acetate, (2) from 5 to 50 percent of a heat-hardenable resin obtained by condensing a phenol selected from the class consisting of phenol, cresol, xylol and mixtures thereof, with formaldehyde in the ratio of one mol of the phenol to 0.7 to 2 mols of the formaldehyde in the presence of an alkaline catalyst, (3) from 0.3 to 1.2 percent, based on the weight of resin solids represented by the polyvinyl formal resin, of a condensation product selected from the group consisting of urea-aldehyde, alkylated urea aldehyde, pyrrole-aldehyde, aromatic amine aldehyde, and thiourea-aldehyde condensates, and (4) a solvent in which (1), (2) and (3) are soluble composed of a mixture of cresol and naphtha, the solids content of the treating solution for the conductor being composed, by weight, of from 5 to 25 parts of the above-described resinous ingredients to about 75 to 95 parts of the cresol naphtha solvent. 10 15 20 25 30

2. The insulated electrical conductor of claim 1 in which the condensation product contained in the insulation comprises a butylated urea-formaldehyde condensate.

3. The insulated electrical conductor of claim 1 in which the condensation product contained in the insulation comprises trimethylol urea.

4. The insulated electrical conductor of claim 1 in which the condensation product in the insulation comprises a pyrrole-formaldehyde condensate.

5. The insulated electrical conductor of claim 1 in which the condensation product contained in the insulation comprises an aniline-formaldehyde condensate.

6. The insulated electrical conductor of claim 1 in which the condensation product contained in the insulation comprises an aniline-acetaldehyde condensate.

#### References Cited in the file of this patent

##### UNITED STATES PATENTS

|           |                |               |
|-----------|----------------|---------------|
| 2,239,441 | D'Alelio       | Apr. 22, 1941 |
| 2,290,675 | D'Alelio       | July 21, 1942 |
| 2,292,333 | D'Alelio       | Aug. 4, 1942  |
| 2,292,334 | D'Alelio       | Aug. 4, 1942  |
| 2,307,588 | Jackson et al. | Jan. 5, 1943  |
| 2,466,399 | Dunlop         | Apr. 5, 1949  |
| 2,687,385 | Olson          | Aug. 24, 1954 |
| 2,730,466 | Daszewski      | Jan. 10, 1956 |

##### FOREIGN PATENTS

|         |           |               |
|---------|-----------|---------------|
| 144,220 | Australia | Nov. 14, 1951 |
|---------|-----------|---------------|